

1

2,834,659

## CHEMICAL POLISHING OF METALS

Owen B. Mathre and Donald M. Sowards, Wilmington, Del., assignors to E. I. du Pont de Nemours and Company, Wilmington, Del., a corporation of Delaware

No Drawing. Application March 25, 1957  
Serial No. 647,980

8 Claims. (Cl. 41—42)

This invention relates to the chemical polishing of metals; more particularly it relates to the chemical treatment of metals to impart thereto a smooth, bright polished surface.

Many attempts have been made heretofore to produce polished surfaces on metals, particularly copper and aluminum and their copper-rich or aluminum-rich alloys, by dipping in various combinations of chemicals. Somewhat attractive results have been obtained by such use of phosphoric acid alone or in combination with substances including acetic acid, sulfuric acid, chromic acid, and hydrogen peroxide.

Such previously-known processes were not altogether satisfactory for several reasons, for example, they imparted insufficient brightness, they caused etching and pitting, the solutions were highly unstable and could not be satisfactorily regenerated.

It is an object of this invention to provide an improved process for the chemical polishing of metals.

It is another object of this invention to provide an improved highly stable polishing composition for the chemical polishing of metals, which composition may be readily regenerated.

It is still another object of this invention to provide an improved process for the chemical polishing of copper, copper-rich alloys, aluminum, and aluminum-rich alloys.

Other objects of this invention will appear hereinafter.

The objects of this invention may be achieved, in general, by contacting a metal surface with a solution containing monoperphosphoric acid, ortho-phosphoric acid and water at a temperature between 90° C. and 130° C.

The content of monoperphosphoric acid,  $H_3PO_5$ , in the solution should preferably be between 0.3 and 5.4 percent, the ortho-phosphoric acid between 70 and 80 percent, and the water between about 15 and 25 percent, and to obtain optimum results the solution should contain 0.5% to 3% monoperphosphoric acid, 73% to 79% ortho-phosphoric acid, and 18% to 23% water. Although generally not present in ortho-phosphoric acid, the presence of meta- or pyro-phosphoric acid is not objectionable.

The contact or treatment time of the metal surface with the solution is from ten seconds to four minutes and preferably between thirty seconds and one and one-half minutes. The temperature of treatment should preferably be within the range 90° C. to 110° C.

The metal object after treatment by immersion, spraying, brushing, or the like, is removed and rinsed with water which preferably contains 1/4% to 1% nitric acid, after which it is dried. The drying may be carried out at room temperature or at an elevated temperature, preferably below about 100° C.

Metals which are most readily polished by the process of this invention include aluminum, aluminum-rich alloys, i. e., alloys containing in excess of 50% aluminum, copper, copper-rich alloys, i. e., alloys containing at least

2

50% copper, e. g., brass, German silver, bronze, and the like.

The metals, prior to contact with the polishing solutions of this invention if soiled may be cleaned and de-greased in a manner well known in the art.

The polishing solutions of this invention are quite stable and may be maintained at the requisite strength or regenerated to top strength by the simple addition of the required amounts of the ingredients to produce the composition ranges above set forth. Aluminum or magnesium, dissolved from alloys, may be contained in the polishing solution up to 3% without noticeable effect on the stability of the solution. Dissolved copper, however, will reduce the stability of the bath. If the copper content exceeds about 1% of the solution it may be desirable to discard the solution rather than regenerate the same by addition of monoperphosphoric acid.

The following examples are given to illustrate the details of the invention, it being understood that the specific details set forth therein are not necessarily limitative of the invention.

### Example I

A clean brass strip having the approximate composition of 67% copper and 33% zinc is immersed in a solution composed of

|                                      | Percent |
|--------------------------------------|---------|
| Commercial 85% ortho-phosphoric acid | 77      |
| Monoperphosphoric acid               | 2       |
| Water                                | 21      |

and having a temperature of about 100° C. for fifteen seconds. The strip is immediately rinsed with clean, cold tap water and dried at room temperature. The brass strip is visibly brightened to remarkable extent from a rather dull appearance to an appearance resembling a mirror.

The following five examples show the polishing of strips of aluminum alloy 1100 containing the following approximate analysis: 1.0% silicon and iron, 0.2% copper 0.05% manganese, 0.10% zinc, 0.15% other metals, 99.0% min. aluminum. The compositions and temperatures of the polishing solutions, the period of immersion, and the gloss of the polished aluminum are tabulated in these examples. The gloss measurements were made on a Hunter multipurpose reflectometer. The mirror supplied with the instrument was used as a secondary standard with a gloss value of 10.0. This gloss of the mirror was checked against a black gloss standard and the value obtained was within experimental error. In each example the aluminum strips, after treatment in the polishing solution, were rinsed with cold tap water and dried at room temperature.

| Example | Solution Composition (Percent)                                                                    | Soln. Temp. (°C.) | Time of Immersion (seconds) | Gloss      |
|---------|---------------------------------------------------------------------------------------------------|-------------------|-----------------------------|------------|
| II      | Ortho-phosphoric acid, 80.8<br>Monoperphosphoric acid, 2.4<br>Water, 16.8                         | 93<br>97          | 60<br>60                    | 9.3<br>9.6 |
| III     | Ortho-phosphoric acid, 81.2<br>Monoperphosphoric acid, 1.9<br>Water, 16.1<br>Dissolved Metal, 0.8 | 108<br>103        | 30<br>60                    | 8.4<br>9.7 |
| IV      | Ortho-phosphoric acid, 72.2<br>Monoperphosphoric acid, 2.4<br>Water, 25.2<br>Dissolved Metal, 0.2 | 96<br>100         | 60<br>60                    | 8.3<br>9.3 |
| V       | Ortho-phosphoric acid, 78.4<br>Monoperphosphoric acid, 1.8<br>Water, 19.6<br>Dissolved Metal, 0.2 | 103<br>101        | 90<br>30                    | 9.3<br>7.5 |
| VI      | Ortho-phosphoric acid, 74.9<br>Monoperphosphoric acid, 1.7<br>Water, 23.2                         | 100<br>96         | 60<br>30                    | 8.6<br>6.1 |

The following example discloses the polishing of aluminum alloy No. 5357 having the following composition: 0.12% silicon, 0.17% iron, 0.07% copper, 0.15-0.45% manganese, 0.8-1.2% magnesium, 0.15% other metals, remainder aluminum. The polishing procedure employed was the same as above described in Examples II to VI.

*Example VII*

|                                          | °C. | Sec. | Gloss |
|------------------------------------------|-----|------|-------|
| Ortho-phosphoric acid, 75.8 percent..... | 103 | 60   | 9.6   |
| Monoperphosphoric acid, 2.7 percent..... | 105 | 60   | 9.2   |
| Water, 21.4 percent.....                 | 103 | 30   | 7.8   |

Similar polishing was obtained by treating aluminum alloys Nos. 1175, 3003 and 6063 in solutions of the kind disclosed in the above examples. These aluminum alloys have the following compositions:

Alloy 1175:  
0.15% silicon+iron  
0.10% copper  
99.75% min. aluminum

Alloy 3003:  
0.6% silicon  
0.7% iron  
0.2% copper  
1.0-1.5% manganese  
0.1% zinc  
0.15% other metal  
Remainder—aluminum

Alloy 6063:  
0.2-0.6% silicon  
0.35% iron  
0.10% copper  
0.45-0.9% magnesium  
0.10% chromium  
0.10% zinc  
0.10% titanium  
0.15% other metal  
remainder—aluminum

The polishing compositions of the present invention are fast acting, non-pitting, stable compositions which are readily maintained or brought up to requisite treatment strength.

The treatment of metal surfaces can be carried out on metal objects having quite irregular surfaces to produce a uniform polished appearance.

Throughout the specification and claims, any reference to parts, proportions and percentages refers to parts, proportions and percentages by weight unless otherwise specified.

Since it is obvious that many changes and modifications can be made in the above-described details without departing from the nature and spirit of the invention, it is to be understood that the invention is not to be limited to said details except as set forth in the appended claims.

We claim:

1. A metal polishing composition containing 0.3% to 5.4% monoperphosphoric acid, 70% to 80% phosphoric acid, and 15% to 25% water.
2. A metal polishing composition containing 0.5% to 3% monoperphosphoric acid, 73% to 79% phosphoric acid, and 20% to 23% water.
3. The process of polishing a metal surface which comprises contacting the same at a temperature of 90° C. to 130° C. with a solution containing monoperphosphoric acid, a phosphoric acid, and water.
- 25 4. The process of polishing a metal surface which comprises contacting the same at a temperature of 90° C. to 130° C. with a solution containing 0.3% to 5.4% monoperphosphoric acid, 70% to 80% phosphoric acid, and 15% to 25% water.
- 30 5. The process of polishing a metal surface which comprises contacting the same at a temperature of 100° C. to 110° C. with a solution containing 0.5 to 3% monoperphosphoric acid, 73% to 79% phosphoric acid, and 20% to 23% water.
- 35 6. The process of claim 3 in which the metal is from the group consisting of aluminum, aluminum-rich alloys, copper, and copper-rich alloys.
- 40 7. The process of claim 4 in which the metal is from the group consisting of aluminum, aluminum-rich alloys, copper, and copper-rich alloys.
8. The process of claim 5 in which the metal is from the group consisting of aluminum, aluminum-rich alloys, copper, and copper-rich alloys.

No references cited.

UNITED STATES PATENT OFFICE  
CERTIFICATE OF CORRECTION

Patent No. 2,834,659

May 13, 1958

Owen B. Mathre et al.

It is hereby certified that error appears in the printed specification of the above numbered patent requiring correction and that the said Letters Patent should read as corrected below.

Column 3, under the heading "Alloy 6063:" following "0.10% copper"  
insert -- 0.10% manganese --.

Signed and sealed this 15th day of July 1958.

(SEAL)

Attest:

KARL H. AXLINE

Attesting Officer

ROBERT C. WATSON  
Commissioner of Patents